

[54] WARP KNIT DENIM FABRICS

[75] Inventor: Bascum G. Lesley, Pickens, S.C.

[73] Assignee: Deering Milliken Research Corporation, Spartanburg, S.C.

[22] Filed: Aug. 13, 1974

[21] Appl. No.: 496,952

[52] U.S. Cl. .... 66/195

[51] Int. Cl.<sup>2</sup> .... D04B 21/00

[58] Field of Search .... 66/190-195

[56] References Cited

UNITED STATES PATENTS

2,040,058 5/1930 Mendel et al. .... 66/176  
2,114,004 4/1938 Reinthal .... 66/195

FOREIGN PATENTS OR APPLICATIONS

70,964 1/1970 Germany  
61,836 5/1968 Germany .... 66/195

OTHER PUBLICATIONS

Weigkricht, "Bindungslehre Kettenwirkerei," 1 Teil, 1950, p. 15, Abb. 55.

Weigkricht, "Bindungslehre der Kettenwirkerei," 1

Tiel, 1953, pp. 11, 24, 27, Abb. 50.  
2 Glanzstoffag Construction Sheets.

Primary Examiner—Ronald Feldbaum  
Attorney, Agent, or Firm—Luke J. Wilburn, Jr.; H. William Petry

[57] ABSTRACT

Warp knit denim fabrics wherein differentially colored or colorable yarn sets or groups are knit together in a fabric having a dominant, typically darker, color forming a background wherein flecks of a less dominant, typically lighter, color are present substantially uniformly throughout the surface of the fabric, thereby giving a fabric whose visual appearance is similar to woven denim fabrics, but which possesses superior fabric qualities. After knitting, the differentially colorable yarn sets may be dyed to selectively color one or more of the yarn sets. The denim effect may be enhanced by sanding or napping the denim surface of the fabric to abrade and/or break the dominant color yarns and blend the lighter color therewith. The fabric may be thereafter calendered, and finished in conventional manner.

16 Claims, 10 Drawing Figures



FIG. 3



FIG. 4



FIG. 1



FIG. 2





FIG. 5



FIG. 6



FIG. 7



FIG. 8



FIG. 9



FIG. 10

## WARP KNIT DENIM FABRICS

This invention relates in general to denim fabrics, and more specifically to warp knit denim fabrics.

Historically, denims have been produced from yarn-dyed spun yarns of cotton or combinations of cotton and synthetic blend spun yarns, which have been woven together to provide a fabric having a generally uniform appearance usually provided by a darker basic color throughout in which small flecks of a lighter color are substantially uniformly dispersed, thereby providing a substantially uniformly appearing fabric of colors somewhere between the darker and lighter colors. Such woven fabrics are typically quite stable, exhibiting little extensibility or stretch to accommodate body movement in garments made from such fabrics. When such woven fabrics include a substantial amount of cotton or other similar yarns, they are quite susceptible to wrinkling, and therefore do not provide preferred characteristics such as ease of care and a long lasting neat appearance.

## BRIEF SUMMARY OF THE INVENTION

It is, therefore, an object of this invention to provide a denim fabric which overcomes the above-noted disadvantages. The present invention provides a denim fabric having good wrinkle resistance and improved extensibility or stretch to better accommodate body movement and provide comfort in garments made thereof, both of which contribute to the ease of care and long lasting neat appearance of such fabrics. Furthermore, the fabrics of the present invention may be piece dyed, as distinguished from the prior art wherein denim fabrics were typically made from yarn dyed yarns.

The foregoing objects and others are provided in accordance with the present invention which is a warp knit denim fabric wherein differentially colored or colorable yarns are knit together to provide a fabric wherein a dominant, typically darker, color forms a background and wherein flecks of a less dominant, typically lighter, color are present substantially uniformly throughout the surface of the fabric, thereby giving a fabric whose visual appearance is similar to woven denim fabrics, but which possesses the improved fabric qualities mentioned above. After knitting, the differentially colorable yarns may be dyed to selectively color one or more of the yarn groups as desired. The denim effect may be enhanced by sanding or napping the denim surface of the fabric to raise the dominant colored yarns and blend the lighter colored yarns therewith.

## BRIEF DESCRIPTION OF THE DRAWINGS

For a better understanding of the invention as well as other objects and further features thereof, reference is made to the following detailed disclosure of preferred embodiments of the invention taken in conjunction with the accompanying drawings thereof, wherein:

FIG. 1 is a photomicrograph of the technical back side of a finished fabric made according to the present invention.

FIG. 2 is a photomicrograph of the technical back side of a fabric knit, dyed, and sanded according to the present invention, but before calendering and finishing.

FIG. 3 is a photomicrograph of the technical back side of a fabric knit and dyed according to the present

invention, but before being sanded, calendered, and finished.

FIG. 4 is a photomicrograph of the technical back side of a greige fabric of the present invention.

5 FIG. 5 is a point diagram illustrating the bar movement patterns by which each of three yarn groups or sets are knit into a fabric of the present invention.

10 FIG. 6 is a point diagram showing in superimposed form, the stitch patterns or bar movements by which the three yarn groups or sets of FIG. 5 are knit together to form fabric according to the present invention.

15 FIG. 7 is a point diagram showing the relationship between a yarn group or set of the ground fabric and a yarn group or set knit therewith to produce the desired denim effect.

20 FIG. 8 is a point diagram, partially schematically illustrating the bar movement of the ground structure yarns and the resultant relationship between the lap portions of the ground structure yarns and the exposed lap portions of the effect yarn sets knit therewith to produce the desired denim effect.

25 FIG. 9 is a point diagram showing individual bar movement patterns by which each of four yarn groups or sets are knit into a fabric according to the present invention.

30 FIG. 10 is a point diagram showing in superimposed form, the stitch or bar movement patterns by which the four yarn groups or sets of FIG. 9 are knit together to form fabric according to the present invention.

## DETAILED DESCRIPTION OF THE PREFERRED EMBODIMENTS

The warp knit denim fabrics of the present invention are made by knitting differentially colored or colorable yarns together on a warp knitting machine to provide a substantially uniform ground fabric into which other yarns are especially knit to provide the desired denim effect. After knitting, if the differentially colored or colorably yarns are not already of the desired color, the fabric may be dyed to selectively color one or more of the differentially colorable yarns. After the fabric has the desired color, the denim effect may be enhanced by napping or sanding the denim surface of the fabric to further accentuate the similarity in appearance between the inventive warp knit denim fabrics of the present invention to known and esthetically acceptable woven denim fabrics.

40 A preferred way of making the warp knit denim fabrics of the present invention is to knit at least two differentially colorable or colored yarn groups, hereinafter referred to as types, together using the stitch pattern

Bar 1: 6-8, 2-0 (fully threaded to approximate fabric width)

55 Bar 2: 4-2, 0-0 (threaded one-in, one-out)

Bar 3: 4-4, 0-2 (threaded one-out, one-in)

the stitch pattern being given in Raschel designations. One type of yarns is knit according to the Bar 1 pattern, and the Bar 1 yarns thereby form a knit ground fabric structure. The other type yarns are alternately knit in

60 two sets by the Bar 2 and Bar 3 patterns, respectively, those yarns providing the denim effect in conjunction with the aforementioned ground fabric. The number of ends of each yarn set knit by each of the Bar 2 and Bar 3 patterns is only half of the number of ends of the set of yarns knit by the Bar 1 pattern. The inventive fabric is achieved by knitting the fabric on a warp knitting machine having at least three guide bars and one needle bar (such as tricot or Raschel machines) with Bar 1

fully threaded to the approximate width of the desired fabric with the ground structure yarns, and Bars 2 and 3 threaded one-in, one-out and one-out, one-in, respectively, with the effect yarn.

The alternation of the yarns placed in the fabric by the Bar 2 and Bar 3 movement patterns is best illustrated in FIGS. 5 and 6. FIG. 5 indicates separately the movements of the three bars, with the yarns of the Bar 1 ground structure designated 11, and the Bar 2 and Bar 3 effect yarns respectively designated 12 and 13. FIG. 6 shows the three bar movement lines combined in a small section of the fabric schematically illustrated. Each of the yarn sets 12 and 13 shown in FIG. 6 alternately knits, or forms loops, and lays-in their lap portions in successive courses, and both yarns knit alternately in succeeding courses in the same wale, but only in every other wale across the fabric. For example as illustrated in FIG. 6, each of yarns 12 and 13 knit, or form loops, in wales A, C, E, but neither yarn 12 nor yarn 13 knits in wales B, D, F. While each of the yarns illustrated in FIGS. 5 and 6 repeats its knit pattern every two courses, as illustrated in courses I and II, a greater length of the pattern of each yarn, per FIG. 5, and the combined stitch pattern for the fabric, per FIG. 6, have been illustrated for purposes of greater clarity. Thus, it can be seen that the yarns of fully threaded Bar 1 knit in every course, while the yarns of half-threaded Bars 2 and 3 knit in every other course with Bar 2 knitting while Bar 3 is laying in, and vice versa.

As one skilled in the art of warp knitting will recognize, the fabric described above in conjunction with FIGS. 5 and 6 is typically produced by preparing three warps for knitting on a warp knitting machine, such as a tricot or Raschel machine. A first warp set including a number of yarn ends which corresponds approximately to the number of wales desired in the resultant fabric is mounted on the machine and the yarns are threaded through the first guide bar so that a separate end of yarn is threaded through each guide blade on the first guide bar. Second and third warp sets are prepared, each having half as many ends of yarn thereon as the first warp set, and the second and third warp sets are mounted on the knitting machine. Yarns from the second warp set are threaded through the second guide bar so that every other guide blade of the second guide bar is threaded with a separate yarn. Similarly, yarns from the third warp are threaded through the third guide bar so that every other guide blade of the third guide bar, out of phase with the second guide bar by one guide blade, is threaded with a separate yarn. The machine is equipped with the appropriate pattern chains or cams to operate the three guide bars in accordance with the stitch pattern or combination of bar movement patterns described above in conjunction with FIGS. 5 and 6. During knitting, yarns from the first bar are simultaneously pulled into loops, or knitted, on every needle across the desired fabric width on every knitting cycle of the needle bar, and each yarn end is knitted on only two non-adjacent needles in successive cycles of the needle bar. Although the three yarn warp sets have been described as being fed from separate warp beams, the second and third effect yarn sets could be fed from a single warp beam of yarns by doubling the number of ends on the beam if desired.

At the same time, the second and third warp sets of yarns are also knit into the fabric, the yarns from the second and third sets forming a plurality of pairs of yarns, one yarn of each pair coming from the second

warp set and the other yarn of each pair coming from the third warp set. The yarns forming of each pair knit on every other needle of the needle bar across the desired fabric width, such that the combination of the two warp sets provides consecutive loops on every other needle during the knitting cycle. During knitting, a yarn from each pair of yarns knits only on a single needle of the needle bar, alternately knitting and then laying in on succeeding knitting cycles. At the same time the other yarn of each pair knits only on the same needle as the first yarn of the pair alternately knitting and laying in on succeeding knitting cycles, such that, when the first yarn of the pairs knits, the second yarn of the pairs lays in. Therefore, the sets of yarns of the second and third warps are alternately knitting on courses on every other wale throughout the fabric while the first warp yarn set is knitting on every course and every wale, throughout the fabric.

As seen in FIG. 6, the yarns 11 of the warp set forming the ground structure of the fabric describe substantially identical, parallel paths through the fabric. Similarly, the yarns 12 of the first set of effect yarns describe substantially identical, parallel yarn paths throughout the fabric differing from the ground structure yarns, while the yarns 13 of the second set of effect yarns describe substantially identical, parallel paths throughout the fabric differing from those of the other two sets.

While FIGS. 5 and 6 systematically illustrate the stitch patterns that the yarns individually and collectively take in the fabric of the present invention, FIGS. 7 and 8 better illustrate their final relationship and how the stitch patterns of FIGS. 5 and 6 produce the desired denim effect. FIG. 6 shows three courses I, II, I', in which a representative portion of ground yarn 11 and a corresponding representative portion of the effect yarn 12 are isolated to better illustrate their interrelation both during knitting, and as the resultant fabric comes off the knitting machine. During knitting, both yarns 11 and 12 are knit into a loop in wale I. Then yarn 11 passes over three spaces between the needles whereupon it is again knit into a loop in course II. However, in wale B, the effect yarn 12 is laid into the fabric without being pulled into a loop in course II, thereby avoiding being knit but forming a long lap which is laid in at the time and place that the ground yarn 11 is being knit in course II. Then in course I', both yarns are again knit into loops in positions corresponding to the positions in which they were knit into loops in course I. Since the ground yarn in Bar 1 of the knitting machine is knit in course II, wale B, but the effect yarn 12 in Bar 2 of the knitting machine is not knit but the lap portion is laid in about the needle at course II, wale B, that laid-in lap portion of yarn 12, here labelled 14, appears on the technical back surface of the fabric and has a tendency to move laterally (as indicated by arrows 15) when the fabric is taken off the knitting elements of the knitting machine, so that it more naturally aligns itself between the two points at which yarn 12 is knit in wale A. This resultant position of the laid-in lap portion of the effect yarn 12 is indicated by the dashed line at 12'. Since the stitch pattern of the Bar 3 yarn is a mirror image of the stitch pattern of the Bar 2 yarn, except that in the courses where the Bar 2 yarn knits, the Bar 3 yarn lays-in, and vice versa, it will be appreciated that the laid-in lap portions of the Bar 3 yarn behave similarly, with respect to corresponding portions of the ground yarn 11.

This result is illustrated over a wider area in FIG. 8, wherein the short exposed lap portions of effect yarns 12 and 13, illustrated as dashed lines 12' and 13', create the desired denim effect by periodically appearing on the technical back surface over the yarns of the ground fabric. FIG. 8 also shows that these short exposed portions of the effect yarns 12' and 13' are aligned generally parallel to the wales of the fabric. This latter point is particularly advantageous in the present invention, because it allows the knit fabric, as schematically illustrated in FIG. 8, to be passed through a fabric sanding machine or over a fabric napping machine to raise the surface of the fabric in a direction parallel to the wales by breaking and/or abrading filaments of the ground yarns which extend across the wales while causing only a minimal effect in the small exposed portions of the effect yarns because they are generally parallel to the wales of the fabric. During napping or sanding it is the long laps of the ground yarn 11, which extend between and across the space defined by each alternate pair of wales in which the effect yarns are knit, which are sanded or napped up to thereby enhance the desired background color. Such a section of a lap of ground yarn 11 is shown at 16 in FIG. 6.

As previously mentioned certain further surface characteristics may be obtained in the fabric, if desired, by various treatments of the fabric after its formation. The surface of the fabric may be mechanically contacted as by sanding or napping to give it a more suede like appearance and to blend the different colors of the fabric. Preferably, the technical back surface of the fabric may be abraded or the filaments thereof broken (in multifilament yarn constructions) on conventional sanding and napping equipment. Typical of such equipment for sanding is a Curtin Hebert wide face finishing machine model 710, while napping may be accomplished with a Woonsocket Napper. Calendering of the sanded or napped fabric further assists in blending the colors on the surface of the fabric.

The colored and/or colorable yarns suitable for use in the present invention may include any textile yarns which may be knit on a warp knitting machine. The fabrics shown in FIGS. 1-4 of the drawings are composed of continuous filament yarns, the filaments of which may be abraded and/or broken in the mechanical napping or sanding operation; however, spun yarns may also be employed to provide the denim fabric of the present invention. These yarns may also be mechanically raised by sanding or napping if desired. In classic woven denims, the background color is usually darker than the effect color, which if reproduced in the warp knit denim fabric of the present invention would dictate that the ground yarn 11, would typically be a dark yarn, for example a dark blue yarn, and the effect yarns of bars 2 and 3 would be a light yarn, for example a white yarn. However the present invention also includes the use of differentially colorable yarns, which may be selectively dyed after they have been knit in the desired fabric. For example, a yarn which is a cationic dye acceptor might be used as the ground yarn, while a non-cationic dye acceptor yarn is used as the effect yarn. Thus the ground color could be placed in the knit fabric by dyeing it with a cationic dye to produce the desired color, while leaving the yarn forming the effect color, or lack thereof, in its original state. For example, one combination of yarns particularly preferred for use in the presently claimed invention is a cationic dyeable

polyester yarn as the ground yarn and non-cationic dyeable polyester yarn as the effect yarn. The yarns may be textured, if desired.

A representative fabric of the presently claimed invention is illustrated at four different stages, in FIGS. 1-4. FIG. 1 is a photomicrograph of the technical back side of a blue and white polyester fabric of the present invention, which has been dyed, sanded, finished and calendered, to give a desired warp knit denim effect. FIG. 2 is a photomicrograph of the fabric which has been dyed and sanded, but not finished and calendered. FIG. 3 shows the fabric after dyeing only. The uniformity of the fabric surface can be seen to be enhanced by the mechanical surface treatment. FIG. 4 is a photomicrograph of a fabric of the present invention in the greige, before the subsequent steps mentioned above, simply showing the relationship of the yarns, without the benefit of differential coloration. The particular appearance desired in the resultant fabric will dictate the subsequent processing steps, e.g., whether the fabric is merely dyed, dyed and abraded, dyed, abraded and calendered, before finishing.

While the foregoing description has been primarily directed to fabrics made according to the stitch pattern illustrated in FIGS. 5 and 6, it will be appreciated that the fabrics of the present invention may be made with still other warp knit stitch patterns. For example, the ground structure may be formed by any one bar stitch pattern wherein the yarn is knit in every course, but floats over at least one, and preferably two or more wales, between the times that it is knit into each course. The ground fabric may be knit having either open loops or closed loops, as desired. This variation is illustrated, for example, in the fabric of FIGS. 9 and 10 wherein two or three different types of yarns are knit together using the stitch pattern:

Bar 1: 8-6, 0-2 (threaded full to the approximate fabric width)

Bar 2: 4-2, 0-0 (threaded one-in, one-out)

Bar 3: 4-4, 0-2 (threaded one-out, one-in)

Bar 4: 0-0, 4-4 (threaded full to approximate fabric width)

said stitch pattern being given in Raschel designations.

Again here yarn of one type coloration is knit according to the Bar 1 pattern to form a ground structure, and another type coloration yarn is alternatively knit by the Bar 2 and Bar 3 patterns to provide a fabric that contains substantially equal numbers of the Bar 1 yarn, and the total Bar 2 and 3 yarns, as previously explained with respect to the fabric illustrated in FIGS. 5 and 6. The fabric of FIGS. 9 and 10 also includes another set of yarns laid in by the Bar 4 pattern, to provide additional stability in the warp knit denim fabric of the present invention. The Bar 4 yarns are entirely laid in and do not come to the fabric surface. Therefore, Bar 4 yarns play no role in the visual denim surface effect, but they are maintained generally within the fabric to give the fabric more stability. Yarns previously discussed for use in Bars 1, 2, and 3, may be used in those bars in the fabric illustrated by FIGS. 9 and 10, while Bar 4 yarns may be of various types, but a colorless yarn, or a yarn similar in color to the ground yarn, is preferable. For example, the fabric of FIGS. 9 and 10 can be made by using cationically dyeable polyester yarns threaded full in Bar 1, non-cationically dyeable polyester yarns threaded one-in, one-out, and one-out, one-in, respectively, in Bars 2 and 3, and a colorless nylon monofilament fully threaded in Bar 4. In both FIGS. 9 and 10,

the Bar 1 yarn is designated 17, the Bar 2 yarn, 18, the Bar 3 yarn, 19, and the Bar 4 yarn, 20. It will of course be appreciated that the fabric of FIGS. 9 and 10 may be made without the Bar 4 yarns, thereby providing a fabric which corresponds to the fabric of FIGS. 4 and 5, except that the ground yarn is knit having open, instead of closed loops. Although the fabrics in the drawings have been described as having a ground structure composed of either open or closed loops, it should be understood that the loops formed by any of the bars may be open or closed or various combinations of open and closed, depending upon the particular characteristics desired in the final product, without departing from the scope of the invention.

The following specific examples are intended to illustrate various preferred embodiments of the present invention.

#### EXAMPLE I

A 56 gauge Mayer Raschel knitting machine capable of knitting on four guide bars is threaded from four warp sets of yarns in the following manner:

Bar 1 (front bar)—Threaded full with 150 denier, 34 filament, Type 92 cationic dyeable textured Dacron (DuPont) polyester yarn. The bar movement is programmed to provide a knitting stitch **8-6, 0-2** and runner length is set at 122 inches per rack (480 courses = one standard rack).

Bar 2 — Threaded one-in, one-out with 150 denier, 34 filament, Type 56 non-cationic dyeable textured Dacron polyester yarn. The bar movement is programmed to provide a knitting stitch of **4-2, 0-0** and runner length is set at 55 inches per rack.

Bar 3 — Threaded one-out, one-in with 150 denier, 34 filament, Type 56 non-cationic dyeable textured Dacron polyester yarn. The bar movement is programmed to provide a knitting stitch of **4-4, 0-2** and runner length is set at 55 inches per rack.

Bar 4 — Threaded full with 20 denier monofilament nylon **6,6** yarn (DuPont) and programmed to provide a knitting stitch of **0-0, 10-10**. The yarns of Bar 4 are laid in with the runner length of 90 inches per rack.

Bars 2 and 3 are gaited to knit on the same needle. The number of ends of yarns supplied to each bar are as follows: Bar 1-**2088**, Bars 2 and 3-**1044** each and Bar 4-**2088**. The knitted fabric is taken away from the needle bar of the knitting machine at 23.4 courses per inch.

After knitting, the fabric is dyed in a single jet Gaston County pressure jet model 3-10-13. The cationic dyeable yarns of the fabric are dyed with a blue cationic dyestuff, while the non-cationic dyeable yarns are undyed and left white. Upon completion of dyeing the fabric is padded, wet through with a 2% Solusoft **100** softener, vacuum extracted, and dried by passing the fabric through a Proctor **4** drum dryer set at 290°F. at approximately 20 yards per minute. The dried fabric is plated into a doff box.

The technical back of the dried fabric is thereafter napped by passing the fabric through a Woonsocket Napper set at the following operating conditions:

|                   |                     |
|-------------------|---------------------|
| Pile Roll         | 200 rpm             |
| Counter Pile Roll | 250 rpm             |
| Feed In           | 29 Yards Per Minute |
| Feed Out          | 30 Yards Per Minute |

After napping the fabric is vacuum extracted and heat set by pin tentering at 350°F. for approximately 2 minutes. The fabric is thereafter calendered at 20 yds./min. on a BF Perkins Schriner Calendar at a nip roll pressure of 50 tons per square inch and a temperature of 350°F. The finished fabric had a weight of 12.0 oz. per linear yard, a course count of 25 courses per inch, a wale count of 34 wales per inch, and a fabric width of 60 to 62 inches, measured from the tenter pin marks.

The resultant finished fabric exhibits a spun yarn-like hand and has a muted blue and white denim fabric look.

#### EXAMPLE II

A warp knit denim fabric according to the present invention is produced on a 56 gauge Mayer Raschel sample machine of 50 inch width. Three guide bars are used, Bar 1 being fully threaded with 1392 ends of 150 denier, 34 filament textured Dacron Type 92 cationic dyeable polyester yarn (DuPont), and Bars 2 and 3 are threaded one-in, one-out, and one-out, one-in, respectively, with 696 ends of 150 denier, 30 filament Kodel Type **41U** non-cationic dyeable textured polyester yarn (Eastman). A fabric is knit using the stitch pattern Bar 1: **6-8, 2-0**; Bar 2: **4-2, 0-0**; and Bar 3: **4-4, 0-2**; with a Bar 1 (front bar) runner length of 113 inches per rack, and Bars 2 and 3 (middle and back bars) each having runner lengths of 50 inches per rack, respectively, with take up gears of 52/106.

The resultant fabric is dyed in accordance with general procedures of Example I. The technical back side thereof is then sanded by passing the fabric through a Curtin Hebert wide face finishing machine, Model 710, the sand roller surface of which moves in a direction parallel to the wales of the fabric. The specific sanding procedure is as follows: The measured fabric thickness before sanding is 39 to 44 mils and entry speed of the fabric is 10 yards per minute. Sanding roll depth setting is 18 mills, entry tension is 8 to 10 lbs. pressure per square inch, and exit tension 8 to 10 lbs. per square inch. Sanding roll speed is 760 rpm and type sanding paper is 220 grit Norton. The fabric makes two passes through the face finishing machine. The sanded fabric is then finished and calendered in accordance with the general procedures of Example I.

The resultant warp knit denim fabric approximates woven denim in appearance, but has greater extensibility, and a much softer hand.

#### EXAMPLE III

A warp knit denim fabric is made on a 56 gauge Mayer Raschel machine, the width of the fabric on the machine being about 74.3 inches. Three guide bars are used, Bar 1 being fully threaded with 2080 single ends of 150 denier, 34 filament Dacron Type 92 cationic dyeable polyester textured yarn. Bars 2 and 3 were threaded one-in, one-out, and one-out, one-in, respectively, with 1040 single ends of 150 denier, 30 filament Kodel Type **41U** non-cationic dyeable textured polyester yarn. The warp knit denim fabric is knit using the stitch pattern of Example I, a Bar 1 runner length of about 113 inches per rack, with Bars 2 and 3 each having a runner length of about 50 inches per rack, respectively. The greige fabric is knit to about 27.8 courses per inch and about 28 wales per inch on the machine, to produce a greige fabric of weight of about 6.0 ounces per square yard on the machine.

The resultant fabric is then dyed as in Example I, and sanded in accordance with the general procedures of Examples II. Thereafter, the fabric is finished and calendered in accordance with the general procedures of Example I. The resultant fabric is a warp knit denim approximating the appearance of woven denim fabrics, but having improved extensibility and hand. 5

## EXAMPLE IV

A warp knit denim fabric is produced on a 56 gauge 10 Mayer Raschel machine, the fabric having a width of about 74.6 inches on the machine. Four bars of the machine are used, Bar 1 being fully threaded with 2088 single ends of the same type yarns of Bar 1 of Example III. Bars 2 and 3 are each threaded one-in, one-out, and one-out, one-in, respectively, with 1044 single ends of the type yarns of Bars 2 and 3 of Example III, and Bar 4 is fully threaded with 2088 single ends of 15 denier monofilament duPont semi-dull nylon. The fabric is knit using the bar movement pattern Bar 1: 8-6, 0-2; 15 Bar 2: 4-2, 0-0; Bar 3: 4-4, 0-2; Bar 4: 0-0, 4-4; the Bar 1 runner length being about 114 inches per rack, Bars 2 and 3 each running in about 51 inches per rack, and the Bar 4 runner length being about 42 inches per rack. This produces a fabric of about 24 courses per inch and 20 28 wales per inch of greige fabric on the machine, the greige weight being about 5.0 ounces per square yard. The fabric is dyed as in Example I. The technical back side of this fabric is then sanded as in Example II, and finished and calendered according to general techniques of Example I. The resultant fabric is a warp knit denim having an appearance similar to woven denim, but having greater comfort extensibility than woven denim fabrics, although not as great extensibility as the fabric of Example II, above. This fabric also has better 25 hand than woven denim fabric.

Although specific components, proportions and arrangements of elements have been stated in the above description of preferred embodiments of this invention, other equivalent components and arrangements of elements may be used with satisfactory results and various degrees of quality, or other modifications may be made herein to enhance the appearance of the fabric. It will be understood that such changes of details, materials, arrangements of parts, and uses of the invention described and illustrated herein, are intended to be included within the principles and scope of the claimed invention. For example, the bar movements of the two bars carrying the effect yarns (bars 2 and 3) could be interchanged within the scope of the present invention, and the inlaid yarns of the fourth set of yarns could be 30 knitted in the fabric if desired.

That which is claimed is:

1. A warp knit fabric comprising in combination; a knitted ground structure comprising a set of similarly colored or colorable yarns disposed in plural, substantially identical paths throughout the structure to form a loop in every wale and in every course, the yarn of each path forming a loop in every course with successive loops being alternately positioned in two non-adjacent wales from course to course, and 35 a plurality of sets of surface effect yarns of lighter color or colorability than said set of ground structure yarns forming loops in the ground structure, 40 60 65 1. the yarns of a first set of the surface effect yarns disposed in plural substantially identical paths throughout the structure to form loops only in

alternate courses, the yarn of each path in said first set forming loops in each alternate course of a single wale and forming inlaid lap portions between said loops, and

2. the yarns of a second set of the surface effect yarns disposed in plural substantially identical paths throughout the structure to form loops only in intervening courses to the courses in which loops of said first set of effect yarns are disposed, the yarn of each path of said second set forming loops in each of said intervening courses of a single wale and forming inlaid lap portions between said loops,

the yarns of said first and second sets of surface effect yarns forming said loops only in every other wale of the ground structure with the paths of all inlaid lap portions of yarns in said first and second sets extending in the same general direction and being exposed on the technical back surface of the ground structure and lying generally parallel to the wales thereof.

2. A warp knit fabric as defined in claim 1 wherein the set of ground structure yarns are knit into the fabric in a stitch pattern defined by the Raschel designations 6-8, 2-0.

3. A warp knit fabric as defined in claim 2 wherein the first set of surface effect yarns is knit into the fabric in a stitch pattern defined by the Raschel designations 4-2, 0-0, and wherein the second set of surface effect 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 995

- bar yarns,
3. half threading, one-out, one-in, out of phase with the threading of said second bar yarns, a third guide bar of the warp knitting machine with a plurality of yarns of said lighter color or colorability, and
4. operating said warp knitting machine to cause said bars to pass about the needles of the warp knitting machine to form a warp knit denim fabric in accordance with the following bar movements defined by the Raschel designations:

|            |          |
|------------|----------|
| First Bar  | 6-8, 2-0 |
| Second Bar | 4-2, 0-0 |
| Third Bar  | 4-4, 0-2 |

5

10

15

20

25

30

35

40

45

50

guide bar of the machine, and wherein said sets are knit by moving the guide bars about the needles in the following pattern defined by the Raschel designations:

|        |          |
|--------|----------|
| Bar 1: | 6-8, 2-0 |
| Bar 2: | 4-2, 0-0 |
| Bar 3: | 4-4, 0-2 |

12. A method as defined in claim 11 wherein the first bar of the knitting machine is moved in a bar movement pattern defined by the Raschel designations 8-6, 0-2.

13. A method as defined in claim 11 comprising the additional step of simultaneously laying in a fourth set of yarns from a fourth guide bar to position the yarns generally crossing the wales of the ground structure.

14. A method as defined in claim 13 wherein a fourth set of yarns is laid into the fabric in a bar movement pattern defined by the Raschel designations 0-0, 4-4.

15. A method of manufacturing a warp knit denim fabric, comprising: simultaneously knitting on a warp knitting machine having one needle bar and at least three guide bars,

1. a first warp comprising a plurality of similarly colored or colorable yarns, with an individual yarn from said warp knitting on each needle across the desired fabric width on every cycle of the needle bar and alternating, between only two non-adjacent needles in successive cycles of the needle bar, and

2. second and third warps, each comprising a plurality of surface effect yarns lighter colored or colorable from said first warp, the yarns from said second and third warps forming pairs of yarns, one yarn of each pair coming from said second warp and the other coming from said third warp, the yarns of said pairs knitting on only every other needle across the desired fabric width, one yarn from each of said pairs repeatedly knitting on a needle on one cycle of the needle bar and laying-in on the succeeding cycle of the needle bar, and the other yarn from each of pair repeatedly laying-in on said one cycle of the needle bar, and knitting on said needle during said succeeding cycle of the needle bar.

16. The method of claim 15, wherein the second and third of the three guide bars repeatedly move in a combination of bar movement patterns defined by the Raschel designations: Second Bar: 4-2, 0-0; Third Bar: 4-4, 0-2.

\* \* \* \* \*

55

60

65